

1

2,909,430

## PHOTOGRAPHIC PROCESSES

Howard G. Rogers, Weston, Mass., assignor to Polaroid Corporation, Cambridge, Mass., a corporation of Delaware

No Drawing. Application October 8, 1958  
Serial No. 765,925

15 Claims. (Cl. 96—29)

This invention relates to photography and more particularly to processes for the development of photosensitive silver halide elements.

It is one object of the present invention to provide novel processes for the development of silver halide emulsions, in which the developing agent is capable of developing a photographic latent image and imparting a reversed or positive colored image of said latent image to a superposed image-receiving element.

A further object is to provide novel processes suitable for use in preparing monochromatic and multichromatic photographic images.

Other objects of the invention will in part be obvious and will in part appear hereinafter.

The invention accordingly comprises the processes involving the several steps and the relation and order of one or more of such steps with respect to each of the others which are exemplified in the following detailed disclosure, and the scope of the application of which will be indicated in the claims.

U.S. Letters Patent Nos. 2,559,643 and 2,647,049 to Edwin H. Land disclose examples of diffusion transfer reversal processes wherein a photographic material, such as photosensitive element comprising an exposed silver halide emulsion layer containing a latent image, is processed to impart to an image-carrying or image-receiving element a reversed or positive dye image of said latent image by permeating into said emulsion layer a suitable liquid processing composition and bringing said photosensitive element into superposed relationship with an appropriate image-receiving element.

It has now been discovered that certain compounds, herein referred to as leuco dyes or leuco compounds, are effective as developing agents in diffusion transfer reversal processes such as disclosed in the above-mentioned patents to Edwin H. Land, and, in addition to developing the exposed silver halide emulsion, are effective to impart a positive dye image of the developed silver image to an image-receiving element, as will be further described herein. These leuco compounds are the leuco derivatives of the product of the oxidative coupling of a p-phenylene diamine and a phenolic coupler, as described in detail hereinafter. They are particularly useful in providing the cyan component for a subtractive color process.

In carrying out the process of this invention, a photosensitive element comprising a silver halide emulsion is exposed and a liquid processing composition applied thereto, as by immersing, coating, spraying, flowing, etc., in the dark. In a preferred embodiment, the photosensitive element contains a layer of the leuco compound, and the liquid processing composition is applied to the exposed photosensitive element in a uniform layer as this element is brought into superposed relationship with an image-receiving element. The liquid processing composition permeates the emulsion and provides a solution of leuco compound substantially uniformly distributed therein. As the latent image is developed,

2

the leuco compound is oxidized and immobilized in exposed areas. This immobilization is apparently primarily due to a change in the solubility characteristics of the leuco compound upon oxidation, and especially as regards its solubility in alkaline solutions. The un-oxidized leuco compound retains its solubility in the liquid processing composition, thereby providing an imagewise distribution of unoxidized leuco compound, at least part of which is transferred, by imbibition, to a superposed image-receiving element, said transfer substantially excluding oxidized leuco compound. The latter element receives a depthwise diffusion, from the emulsion, of unoxidized leuco compound without appreciably disturbing its imagewise distribution, thereby giving a reversed or positive, colored, image of the developed negative image. The image-receiving element may contain agents adapted to oxidize, mordant or otherwise fix the diffused, unoxidized leuco compound. Imbibition periods of approximately one minute have been found to give good results, but this contact period may be adjusted where necessary to compensate for variations in temperature or other conditions. The desired positive image is revealed by stripping the image-receiving element from the photosensitive element at the end of the imbibition period.

The leuco compounds or leuco dyes disclosed herein may be disposed in the liquid processing composition, in the image-receiving element, or in the photosensitive element; for example, in, on, or behind the silver halide emulsion layer. When employed in either element the leuco dye becomes solubilized by the liquid processing composition as it permeates the element. In a preferred embodiment, a coating or layer of the leuco dye is incorporated in the photosensitive element, preferably behind the silver halide emulsion layer, i.e., on the side of the emulsion adapted to be located most distant from the photographed subject when the photosensitive element is exposed. Placing the leuco dye behind the emulsion layer has the advantage of providing increased contrast in the positive image, and also minimizes any light-filtering action if the leuco dye is colored. If the leuco dye is colorless, it may be incorporated in the silver halide emulsion without adverse light-filtering effect. Where the leuco dye is employed in a layer within the photosensitive element, it may be applied by using coating solutions containing about 0.5 to 8%, by weight, of the leuco dye. Similar concentrations may be used if the leuco dye is utilized as a component of the liquid processing composition.

The liquid processing composition referred to above comprises at least an aqueous solution of an alkaline material, such as diethylamine, sodium hydroxide or sodium carbonate. If the liquid processing composition is to be applied to the emulsion by being spread thereon, preferably in a relatively thin uniform layer, it may also include a viscosity-increasing compound constituting film-forming material of the type which, when spread over a water-absorbent base, will form a relatively firm and relatively stable film. A preferred film-forming material is a high molecular weight polymer such as a polymeric water-soluble ether which is inert to an alkaline solution, as, for example, a hydroxyethyl cellulose or sodium carboxymethyl cellulose. Other film-forming materials or thickening agents may be employed whose ability to increase viscosity is substantially unaffected when left in solution for a long period of time.

The unoxidized leuco dye which diffuses to the image-receiving element is oxidized to provide the desired positive dye image. This oxidation may be effected by merely exposing the stripped image-receiving element to the air. In a preferred embodiment, the image-receiving element has incorporated therein an oxidizing

agent for the purpose of speeding up positive dye image formation and providing full image density immediately upon stripping. The incorporation of an oxidizing agent in the image-receiving element for the purpose of oxidizing unreacted developing agent permeated therein is described in the previously mentioned U.S. Patent No. 2,559,643. As examples of suitable oxidizing agents, mention may be made of peroxy compounds such as sodium or potassium perborate, certain dichromates such as ammonium dichromate, and compounds having polyvalent metallic elements in higher valent form such as copper, iron and cerium, wherein the metallic element is in higher valent form. Examples of these latter mentioned agents are cupric salts such as cupric sulfate. Another suitable oxidizing agent is benzoyl peroxide. Other useful oxidizing agents are quinones, and particularly 2,3-dicyano-1,4-benzoquinone.

As stated above, the leuco developing agents of this invention are the leuco derivatives of the products of the oxidative coupling of p-phenylene diamines with phenolic couplers. The products of such oxidative coupling are commonly referred to in the art as "indo-phenols," but it should be noted that a more precise, although less used, name is "indoanilines." (See Synthetic Dyes, vol. II, K. Venkataraman, Academic Press, Inc., New York, N.Y., 1952, page 763.)

The leuco dyes of this invention may be represented by the formula



wherein Y is a substituted or unsubstituted benzene or naphthalene ring containing a hydroxyl group para to and nitrogen to which Y is attached, each Z may be hydrogen, alkyl, amino or alkoxy, X may be hydrogen or alkyl and each X may be the same or different. As used in this specification, alkyl is intended to include substituted alkyl groups, e.g., sulfonamido-alkyl groups. Y may also be substituted by halogen, alkyl, nitro, cycloalkyl, etc.

It is within the scope of this invention to use these leuco compounds as either the free base or as an acid addition salt, for example, the corresponding hydrochloride or oxalate.

As specific examples of leuco dyes within the scope of this invention, mention may be made of the following:

2 - chloro-4-(4'-diethylamino-2'-methylanilino)-5 - nitro-1-naphthol hydrochloride

2 - chloro-4-(4'-diethylamino-2'-methylanilino)-naphthol hydrochloride

2 - chloro-4-(4'-diethylamino-anilino)-5-nitro-1-naphthol hydrochloride

4-(4'-dimethylamino-anilino)-1-naphthol oxalate

4 - (4'-dimethylamino-anilino)-1-naphthol hydrochloride

2 - chloro-4-[4'-(N-ethyl-N-beta - methylsulfonamidoethyl)-amino-2'-methoxyanilino]-6-cyclohexyl-phenol hydrochloride

4 - (4' - dimethylamino-2'-methylanilino)-5-nitro-1-naphthol hydrochloride

2 - chloro - 4-(4'-diethylamino-2'-methylanilino)-5-p-toluene-sulfonamido-1-naphthol hydrochloride

2 - chloro-4-[4'-(N-ethyl-N-beta - methylsulfonamidoethyl)-amino-2'-methoxyanilino]-5-nitro-1-naphthol

2 - chloro-4-(4'-diethylamino-2'-methylanilino)-5-nitro-1-naphthol

2 - chloro-4-[4'-(N-ethyl-N-beta - methylsulfonamidoethyl) - amino-2'-methoxyanilino]-1-naphthol hydrochloride

10

15

25

30

40

35

45

50

55

60

65

70

75

2 - chloro-4-(4'-diethylamino-2'-propoxy - anilino) - 1-naphthol hydrochloride  
2,4-diamino-4'-hydroxy-diphenylamine hydrochloride  
1 - (beta-methylsulfonamidoethyl)-5-(3'-chloro-4-hydroxyl-1'-naphthylamino) - 2,3-dihydroindole hydrochloride

The following is an example of a use of the leuco dyes in accordance with this invention, and is given as an illustration only:

*Example 1*

A subcoated cellulose acetate film base is coated with a 4% aqueous gelatin solution. After this coating has dried, a coating is applied of a solution comprising 4 g. of 2-chloro-4-(4'-diethylamino-2'-methylanilino)-5-nitro-1-naphthol hydrochloride and 0.4 g. of p-N-benzylaminophenol in 100 cc. of a solution comprising:

|                                      |    |    |
|--------------------------------------|----|----|
| Cellulose acetate hydrogen phthalate | g  | 4  |
| Acetone                              | cc | 80 |
| Methanol                             | cc | 20 |
| Ethyl Cellosolve                     | cc | 1  |

A silver iodobromide emulsion is applied over the layer of leuco developing agent, after which the coated film base is exposed. The exposed, coated film base is wetted with a liquid processing composition comprising:

|                                |    |     |
|--------------------------------|----|-----|
| Water                          | cc | 100 |
| Sodium carboxymethyl cellulose | g  | 4.5 |
| Sodium hydroxide               | g  | 2.0 |
| Phenyl ethyl alcohol           | cc | 1.5 |

as this film base is brought into superposed relationship with an image-receiving element. The image-receiving element is a baryta paper coated with a solution comprising 3% polyvinyl alcohol, 3% partially hydrolyzed polyvinyl butyral and 0.1% copper nitrate in a mixture of 40% isopropyl alcohol and 60% water. After an imbibition period of approximately one minute, the image-receiving element is separated and is found to contain a cyan, positive dye image of the photographed subject.

It will be noted that a conventional silver halide developing agent may be, and in the above example is, incorporated with the leuco dye. This conventional developer is preferably used in a quantity sufficient to accelerate development of the latent image. Use of such a developing agent has been found helpful in improving the tonal range or steps in the positive image. Some of the reacted leuco dye may be oxidized by an energy transfer reaction with oxidized auxiliary developing agent. The preferred auxiliary developing agents are those having a moderate developing potential. Among the developing agents which are preferred for this purpose are p-N-benzylaminophenol, ascorbic acid, p-anilino-phenol, 1-amino-2-naphthol, diethyl hydroxylamine and Metol (p-N-methylamino-phenol).

It has also been found that hypophosphorus acid will improve the tonal range of the positive image obtained by the use of these leuco developing agents. An example of the use of hypophosphorus acid is:

*Example 2*

A photosensitive element is prepared by coating a subcoated cellulose acetate film base with a 4% aqueous gelatin solution. After this coating has dried, a coating is applied of a solution comprising 3 g. of 2-chloro-4-(4'-diethylamino-2'-methylanilino)-5-nitro-1-naphthol hydrochloride and 1% hypophosphorus acid in 33 cc. of methanol and 66 cc. of an acetone solution containing 6% cellulose acetate hydrogen phthalate. After this coating has dried, a silver iodobromide emulsion is applied. An image-receiving element is prepared by coating a baryta paper with a solution comprising 3% partially hydrolyzed polyvinyl butyral and 3% polyvinyl alcohol in a mixture of 40% isopropyl alcohol and 60%

water. The photosensitive element is exposed and a liquid processing composition comprising:

|                                |    |     |
|--------------------------------|----|-----|
| Sodium carboxymethyl cellulose | g  | 4.5 |
| Sodium hydroxide               | g  | 3.0 |
| Metol                          | g  | 0.1 |
| Water                          | cc | 100 |

is applied to the exposed photosensitive element as it is brought into superposed relationship with the image-receiving element. After an imbibition period of approximately one minute, the image-receiving element is separated and contains a cyan positive dye image of the photographed subject.

An example of the use of sulfite with a leuco dye, and given as an illustration only, is:

*Example 3*

A photosensitive element is prepared by coating a sub-coated cellulose acetate film base with a 4% aqueous gelatin solution. After this gelatin coating has dried, a coating is applied of a solution comprising 3 g. of 2-chloro-4-(4'-diethylamino-anilino)-5-nitro-1-naphthol hydrochloride, 33 cc. of methanol and 66 cc. of an acetone solution containing 6% cellulose acetate hydrogen phthalate. A silver iodobromide emulsion is applied over the layer containing the leuco dye. An image-receiving element is prepared as described in Example 2. The photosensitive element is exposed and a liquid processing composition comprising:

|                                |    |     |
|--------------------------------|----|-----|
| Water                          | cc | 100 |
| Sodium carboxymethyl cellulose | g  | 4.5 |
| Sodium hydroxide               | g  | 2.0 |
| Phenylethyl alcohol            | g  | 1.5 |
| p-Anilino phenol               | g  | 0.2 |
| Sodium sulfite                 | g  | 0.5 |

is applied to the exposed photosensitive element as it is brought into superposed relationship with the image-receiving element. After an imbibition period of approximately one minute, the image-receiving element is separated and contains a cyan positive dye image of the photographed subject.

It will be apparent that by appropriate selection of the image-receiving element from among suitable known opaque and transparent materials, it is possible to obtain either a colored positive reflection print or a colored positive transparency. Likewise, the inventive concepts herein set forth are adaptable for multicolor work by the use of special photographic materials, for example film materials of the type containing two or more photosensitized elements associated with a suitable number of image-receiving elements and adapted to be treated with one or more liquid processing compositions, appropriate developing agents suitable to impart the desired subtractive colors being incorporated in the photosensitized elements or in the liquid processing compositions. Examples of such photographic materials are disclosed in the previously mentioned U.S. Patent No. 2,647,049 to Edwin H. Land.

The inventive concepts herein set forth are also adaptable to the formation of colored images in accordance with the photographic products and processes disclosed and claimed in the copending application of Edwin H. Land, Serial No. 448,441, filed August 9, 1954, which is a continuation-in-part of Serial No. 176,961, filed August 1, 1950, and now abandoned, and also those set forth in the copending application of Howard G. Rogers, Serial No. 748,421, filed July 14, 1958, which is a continuation-in-part of Serial No. 415,073, filed March 9, 1954, and now abandoned.

U.S. Patent No. 1,102,028 to Rudolph Fischer, issued June 30, 1914, discloses the silver halide developing ability of leuco compounds such as those disclosed herein, as well as the formation of a dye image by these compounds. The photographic art, however, has general-

ly considered the use of these compounds in color photography to be impractical and undesirable. It was therefore unexpected that these leuco compounds would be useful in obtaining a colored, positive image by a diffusion transfer process such as described herein.

In those instances where the photographic art has referred to the use of these leuco compounds, it has been suggested that the presence of sulfite be avoided. See, for example History of Color Photography, Joseph S. Friedman, American Photographic Publishing Co., Boston, Mass., 1944, p. 374-5. It has been found, however, contrary to these suggestions, that it is not necessary to exclude sulfite when using these leuco compounds, and small amounts of sulfite may be used, particularly where they are employed in a diffusion transfer reversal process such as disclosed herein to obtain a positive dye image.

In the preceding portions of the specifications, the expression "color" has been frequently used. This expression is intended to include the use of a plurality of colors to obtain black.

In employing the leuco compounds of this invention in film units suitable for use in self-developing cameras, such as the Polaroid Land Camera, sold by Polaroid Corporation, Cambridge, Massachusetts, the film unit may comprise a photosensitive element, an image-receiving element adapted to be superposed on said photosensitive element, and a rupturable container holding a processing composition and adapted to release its contents for spreading over predetermined areas of said elements after rupture. Suitable structures of this type are described in the herein-mentioned U.S. patents and patent applications. The leuco compound may be located in the processing composition or in a layer of the photosensitive element.

This application is in part a continuation of my copending U.S. application, Serial No. 464,175, filed October 22, 1954 (now abandoned).

Since certain changes may be made in the above processes without departing from the scope of the invention herein involved, it is intended that all matter contained in the above description shall be interpreted as illustrative and not in a limiting sense.

What is claimed is:

1. In a process of forming photographic images in color, the steps which comprise developing a latent image contained in an exposed silver halide emulsion with an aqueous alkaline solution of a leuco compound of the formula:



60 wherein Y is selected from the group consisting of unsubstituted and substituted benzene and naphthalene rings containing a hydroxyl group in para position to the nitrogen to which Y is attached, each Z is selected from the

65 group consisting of hydrogen, alkyl, amino and alkoxy radicals and each X is selected from the group consisting of hydrogen and alkyl radicals, to thereby provide in said emulsion a predetermined distribution of unoxidized leuco compound, transferring at least part of said distribution of unoxidized leuco compound by imbibition

70 from said emulsion to an image-receiving layer in superposed relationship with said emulsion and oxidizing the diffused, transferred, unoxidized leuco compound to impart to said image-receiving layer a reversed, positive dye image of the developed image.

2. The process as defined in claim 1 wherein said leuco compound is disposed, prior to exposure, in a photosensitive element comprising said exposed silver halide emulsion, and the solution containing said leuco compound is formed by permeating said photosensitive element with an aqueous alkaline liquid capable of solubilizing said leuco compound.

3. The process as defined in claim 2 wherein said leuco compound is present in the photosensitive element as an acid addition salt.

4. The process as defined in claim 3 wherein said acid addition salt is the hydrochloride.

5. The process as defined in claim 2 wherein said liquid is introduced by being spread in a substantially uniform layer between said photosensitive element and said image-receiving layer as said photosensitive element and said image-receiving layer are brought into superposed relationship.

6. The process as defined in claim 2 wherein said liquid contains a thickener for increasing viscosity and for facilitating the spreading thereof between said photosensitive element and said image-receiving layer.

7. The process as defined in claim 1 wherein said leuco compound is dissolved in an aqueous alkaline solution prior to application of said solution to said exposed emulsion.

8. The process as defined in claim 1 wherein the diffused, transferred, unoxidized leuco compound is oxidized by exposure to air.

9. The process as defined in claim 1 wherein said diffused, transferred, unoxidized leuco compound is oxidized by an oxidizing agent incorporated in the image-receiving layer.

10. The process as defined in claim 1 wherein said aqueous alkaline solution contains a silver halide developing agent in addition to said leuco compound.

11. The process as defined in claim 2 wherein hypophosphorous acid is disposed with said leuco compound in said photosensitive element.

12. The process as defined in claim 1 wherein said leuco compound is 2-chloro-4-(4'-diethylamino-2'-methylanilino)-5-nitro-1-naphthol.

13. The process as defined in claim 1 wherein said leuco compound is 2-chloro-4-(4'-diethylamino-anilino)-5-nitro-1-naphthol.

14. The process as defined in claim 1 wherein said leuco compound is 2-chloro-4-[4'-(N-ethyl-N-methylsulfonamidoethyl)-amino-2'-methoxyanilino]-1-naphthol.

15. The process as defined in claim 1 wherein said development is effected in the presence of an accelerating silver halide developing agent.

References Cited in the file of this patent

UNITED STATES PATENTS

|           |          |               |
|-----------|----------|---------------|
| 1,102,028 | Fischer  | June 30, 1914 |
| 2,206,126 | Schinzel | June 2, 1940  |
| 2,559,643 | Land     | July 10, 1951 |
| 2,647,049 | Land     | July 28, 1953 |